

# UNITED STATES PATENT OFFICE.

CHARLES H. ALDRICH AND JOHN K. BRYAN, OF BALTIMORE, MARYLAND, ASSIGNEES TO ELECTROLYTIC ZINC COMPANY, INC., OF NEW YORK, N. Y., A CORPORATION OF NEW YORK.

## ELECTROLYTIC REFINING OF METALLIC ZINC-BEARING MATERIALS.

1,299,414.

Specification of Letters Patent.

Patented Apr. 8, 1919.

No Drawing.

Application filed July 26, 1916. Serial No. 111,350.

To all whom it may concern:

Be it known that we, CHARLES H. ALDRICH and JOHN K. BRYAN, both citizens of the United States, residing at Baltimore, in the 5 State of Maryland, have invented certain new and useful Improvements in Electrolytic Refining of Metallic Zinc-Bearing Materials, of which the following is a specification.

This invention relates to a method of refining metallic zinc-bearing materials by the electrolytic process, and has for its object to obtain a coherent reguline deposit of zinc on the cathode, free from impurity, sponge or moss. These difficulties incident to the 10 deposition of pure zinc are well recognized and various explanations have been offered. One undoubted fact is that since zinc is more electro-positive even than nickel, all the heavy metals must be removed before its 15 deposition is attempted. It has been stated that the sponge was produced chiefly when a weak solution, or a low current-density was used, and that hydrogen was usually evolved simultaneously. The cause of the spongy 20 deposit is variously explained, some authorities ascribing it to the existence of a compound of zinc and hydrogen, while others trace it to the presence of oxid, produced, for example, either by the use of a solution containing a trace of basic salt of zinc, or by 25 the presence of a more electro-negative metal, which, being co-deposited, sets up local action at the expense of the zinc.

In the present process accordingly we 30 have had it in view to secure so far as possible the proper operating conditions to overcome the difficulties referred to, among others, to whatever causes these difficulties may be ascribed.

40 In a typical operation involving the principles of this invention, the zinc-bearing material is cast into anode form, placed in tanks in series circuit, with suitable cathodes, and an electrolyte such as zinc sulfate, preferably containing a small percentage of free sulfuric acid. This electrolyte may be continuously circulated in accordance with any well known or preferred practice so as to 45 avoid segregation within the electrolyte, that is, to maintain the homogeneity of the electrolyte. 50 It has been common practice heretofore in the electrolytic refining of zinc to employ a neutral or basic sulfate solution, which, as indicated above, probably gave rise to some 55 of the various difficulties encountered, such as mossy deposit, non-adherent deposit upon the cathode, and the production of impure cathode zinc. Accordingly, as one of the 60 improvements which we have devised, we employ a slightly acid electrolyte, and have found that the best strength of acid to maintain in the electrolyte is about .1 to about .5 of one per cent. of free sulfuric acid, this 65 acidity being maintained either by the addition of sulfuric acid at intervals or continuously, or by placing insoluble anode tanks in the electrolytic circuit, so that the acid may 70 be regenerated in this manner with the accompanying deposit of metallic zinc, the resultant electrolyte being returned to the regular circuit, thus furnishing the acid required. The limits for the acid as given 75 above are believed to be about the best, but more acid might not be detrimental, and it is 80 possible that less than .1 of one per cent. might be used to good effect in connection with a rapid circulation of the electrolyte, because rapid circulation would probably give smoother deposit and a smooth deposit 85 would probably not dissolve so quickly in the acid. We have found that iron in such a slightly acid electrolyte is not detrimental—on the contrary, it is beneficial as it 90 helps to produce a reguline deposit on the cathode, and does not precipitate on the cathode with the zinc. A possible explanation of this action is that some of the iron may act as an oxidizing agent, to prevent the formation of zinc hydrate, to which some 95 authorities have attributed the formation of zinc sponge. At any rate, we have found that we can allow the iron to reach as high as one gram per liter with good results as to the character of the cathode deposit. Should the iron in solution go above a point which may be determined upon as the danger point, it can be removed by any of the

well known methods, such as precipitation with zinc oxide in a neutral solution. The temperature of the electrolyte we prefer to keep at about 40° C. or lower, as this seems to be the optimum in the light of our experiments thus far, though a somewhat higher temperature might be employed.

We have found that cadmium, which is one of the impurities that gives particular trouble, does not go into solution in the electrolyte, so long as the slime is kept in contact with the excess zinc remaining in the anode, this being due to the fact that cadmium is more electro-negative than zinc. On this account, and for other reasons which will be obvious, we propose to surround the anode with a bag or similar envelop, which may be made of duck, canvas or the like, which bag preferably fits the anode snugly throughout the whole operation. This anode envelop of course prevents the impurities from the anode, which remain as slime, from mechanically contaminating the cathode deposit; and it cuts down the percentage of slime produced, because the slime, being always in contact with the anode, continues to act as part of the anode, and the zinc content of the slime continues to dissolve, due to electrolytic action. It also insures that the cadmium content of this slime remains in close contact with the excess zinc remaining in the anode, and consequently does not go into solution. Furthermore, this close-fitting envelop serves to maintain the integrity of the anode, that is, prevents the dropping off of flakes from the anode, which, in the former practice, would fall to the bottom of the cell and consequently be affected by electrolysis very little, if at all. The form of bag which we prefer to employ, and the means for insuring that the bag shall at all times snugly fit the anode, notwithstanding the gradual disintegration of the anode by electrolysis, is described in an application for Patent, Serial No. 111367, filed July 26th, 1916, in the name of Heber M. Stuart.

Should, by any accident, cadmium go into solution, it can be removed by circulating the electrolyte through a series of insoluble anode tanks for a few hours, the time being dependent on the amount of cadmium present and the current density; since cadmium, being more electro-negative than zinc, will be removed with a portion of the zinc, the resulting electrolyte may then be run back to the main circuit, free from cadmium.

We have also found that it is practicable, where a series of electrolytic tanks are used, in which the usual zinc sulfate electrolytes are flowing continuously from No. 1 tank through the series to No. X tank, using either soluble or insoluble anodes, the impurities, such as cadmium, and particularly this metal, which is detrimental to high grade spelter, may be removed with the cathode

zinc in the first tank of the series, the exact number necessary for the removal of this cadmium, or other metal more electro-negative than zinc, depending on various factors, such as the current density and the amount of the undesired metal in solution. For instance, if the series included twenty tanks we might take out the impure cathode zinc, including the co-deposited undesirable metals, from the first four or five tanks, the cathode zinc in the remaining tanks being free from cadmium or other undesired metals, or at least below the limits allowed for high grade zinc specifications. And this may be done whether soluble or insoluble anodes are employed, so that while, as before stated, we aim to prevent the co-deposition of cadmium or the like by means of the close-fitting envelop for the anode, etc., the method last above described enables us to secure pure cathode zinc as the result of the operation of the cyclic process even though the bag be not used; it being understood that in former practice the impure cathode zinc from the first of a series of tanks was invariably removed and mixed with the purer zinc from the later tanks in the series, the resulting mixture being of course contaminated.

Inasmuch as many changes could be made in the above construction, and many apparently widely different embodiments of our invention could be made without departing from the scope thereof, it is intended that all matter contained in the above description shall be interpreted as illustrative and not in a limiting sense.

It is also to be understood that the language used in the following claims is intended to cover all the generic and specific features of the invention herein described and all statements of the scope of the invention which, as a matter of language, might be said to fall therebetween.

We claim:

1. As a step in the electrolytic separation of metallic zinc-bearing materials in anode form, keeping the cadmium content of such materials out of solution during the electrolysis.

2. As a step in the electrolytic separation of metallic zinc-bearing materials in anode form, keeping the cadmium content of the electrolytically disintegrated anode in contact with an excess of zinc during the electrolysis to prevent the going into solution of the cadmium.

3. As a step in the electrolytic separation of metallic zinc-bearing materials in anode form, keeping the cadmium content of the electrolytically disintegrated anode in contact with the excess of zinc remaining in the anode during the electrolysis to prevent the going into solution of the cadmium.

4. As a step in the electrolytic separation

115

110

120

125

130

of metallic zinc-bearing materials including a metal more electro-negative than zinc and in anode form, keeping the said more electro-negative metal content of the electrolytically disintegrated anode in contact with an excess of zinc during the electrolysis to prevent the going into solution of said more electro-negative metal.

5. As a step in the electrolytic separation  
10 of metallic zinc-bearing materials including a metal more electro-negative than zinc and in anode form, keeping the said more electro-negative metal content of the electrolytically disintegrated anode in contact with the  
15 excess of zinc remaining in the anode during the electrolysis to prevent the going into solution of the said more electro-negative metal.

6. In the electrolytic separation of metallic  
20 zinc-bearing materials in a number of tanks in series circuit, the step which consists in removing the cathode deposit including co-deposited impurities, from the first tank or tanks of the series, and commingling the  
25 cathode deposits from the later tanks of the series, relatively free from such impurities.
7. In the electrolytic separation of metallic zinc-bearing materials, including cadmium, in a number of tanks in series circuit,  
30 the method of recovering substantially cadmium-free cathode zinc which consists in co-depositing cadmium with the zinc in the first tank or tanks of the series, whereby the so-

lution coming to later tanks is relatively cadmium-free and relatively pure zinc is deposited in the later tanks, and segregating the deposits from the first tank or tanks and those from the later tanks.

8. In the electrolytic separation of metallic zinc-bearing materials, including cadmium, in a number of tanks in series circuit,  
40 the method of removing cadmium from the electrolyte which consists in separately treating it electrolytically to cause co-deposition of the cadmium and zinc content, whereby  
45 the solution is relatively freed from cadmium, and then electrolyzing the solution in tanks of the series.

9. In the electrolytic separation of metallic zinc-bearing materials, including cadmium, in a number of tanks in series circuit,  
50 the method of recovering substantially cadmium-free cathode zinc which consists in co-depositing cadmium in a number of the first tanks of the series, the number depending upon the amount of cadmium present, whereby the solution coming to later tanks is relatively cadmium-free and relatively pure zinc is deposited in the later tanks, and segregating the deposits from the first tank or tanks  
55 and those from the later tanks.

In testimony whereof we affix our signatures.

CHARLES H. ALDRICH.  
JOHN K. BRYAN.